

## UNITED STATES PATENT OFFICE

2,016,718

METHOD FOR TREATING BRONZE WASTES  
FOR RECOVERING COPPER, TIN, LEAD,  
AND PRECIOUS METALS THEREFROM

Auguste Hollard, Paris, France

No Drawing. Application November 30, 1931,  
Serial No. 578,224. In France December 1,  
1930

2 Claims. (Cl. 204—57)

This invention relates to a method for treating bronze wastes for recovering copper, tin, lead and precious metals therefrom.

The main object of the invention is to provide 5 an industrial method for treating bronze wastes through electrolysis in order to recover copper, tin, lead and other precious metals contained in the same and to separate them from the sludge formed during the electrolysis.

10 *Separation of copper.*—I do not use smolten bronze anodes because they lead to a progressive impoverishment of the electrolytic bath in copper and I recommend anodes formed of turnings or granulated bronze pressed between two diaphragms and through which passes a flow of air and steam; said flow facilitating the dissolution of the bronze wastes and heating the bath, maintaining it in a suitable circulating condition. Each of these diaphragms is formed of two lead 15 grids—or any other resistant metal—(storage battery grids are most suitable for this purpose) applied against each other, but separated from each other by a sheet of wool (such as for instance a piece of flannel). The electrolysis vat, which 20 may be of wood and the section of which may be a rectangular one, receives said diaphragms, the edges of which are fitted in the bottom and sides of the vat, respectively. Said diaphragms are located at equal distances (a few centimeters) from 25 each other and divide the vat into a number of compartments. The odd compartments receive the bronze wastes and form the anodes which are all connected in parallel. The even compartments receive the cathodes which are all connected in parallel, each cathode being formed of a 30 copper sheet which may be fitted in an insulating frame. Provision is made for the compartments at the ends of the vat to be anodic compartments.

In order to reduce the amount of electric energy given out, the anodic compartments may also 35 be connected in series. The vat will then comprise a first anodic compartment situated at one end of the vat filled with bronze wastes maintained between the outermost wall of the vat and a first diaphragm (double grid, flannel); to this 40 first compartment follows a second one filled with electrolyte and limited by a lead cathode (or of any other resistant metal), on which the electrolytic copper will settle.

45 This cathode forms one of the walls of No. 3 compartment which is an anodic compartment filled with bronze wastes, the other wall of this compartment being a diaphragm (double grid, flannel) limiting No. 4 compartment filled with 50 electrolyte, and so on.

The vat is filled with a solution of copper salt as for instance copper sulphate (150 grams of said salt in a crystallized condition per liter) and of sulphuric acid (100 grams per liter). Thus, the anodes and the cathode are immersed in said solution which is heated by the steam flowing through the compartments and brought to a temperature which may vary for instance between 30 and 60° C. 5

When such temperature is reached, steam addition is usually no more necessary, the temperature being maintained by the passage of the electric current and of the air.

10 The copper precipitates into the cathode in a clean and thick coating under a density of current of 2 to 3 amperes per square decimeter of the cathode.

15 The bath tends to grow poorer in sulphuric acid and such an acid is added to the bath either periodically or continuously. If the concentration of 20 the bath in copper sulphate has a tendency to become greater, the addition of air will be diminished.

25 *Sludge treatment.*—The bronze wastes in the anodic compartments are washed from time to time with water, through which the sludge accompanying the wastes is caused to sink into the bottom of the vat. To this end the vat is first emptied, then the sludge, carried away with the water, passes through a hole provided in the bottom of each compartment and having its bung taken out for this purpose.

30 The sludge is washed out with water and deprived of all copper sulphate which accompanies it, whereafter it is dried and then passed through 35 a sieve (No. 75-100). The pieces remaining on the sieve are treated anew electrolytically with the wastes. The sludge is roasted at a temperature not exceeding 200 to 300° C., as otherwise the copper might be converted into copper protoxide 40 which is insoluble in diluted sulphuric acid and silver might be converted into silver oxide which is soluble in the same acid. After said roasting the sludge is treated by diluted and hot sulphuric acid, for instance 35 liters of sulphuric acid of 66° 45 Bé. and 350 liters of water for 100 kilos of dry sludge. A liquid is thus obtained in which copper sulphate crystallizes in a cold condition. The sulphate which still adheres to the sludge is separated by washing the sludge with water which 50 dissolves the sulphate and the poor copper solution thus obtained is used for subsequent treatments.

55 The sludge extracted and deprived of its copper sulphate is roasted anew in the same condi-

tion and then treated by an acid of  $\frac{1}{10}$  concentration as before, but in a lower quantity. A solution is then obtained which is less concentrated than the first one. The whole is then washed with water and may be roasted once more; after treating with diluted sulphuric acid, a new but very small quantity of copper sulphate is obtained. The residual sludge, which generally does not represent half of its original weight, is dried, ground and smelted with a mixture of rosin and smolten borax in the form of a powder. The rosin allows of a smelting at a temperature which is much lower than the temperature required when using coal. For instance, 10 kilos of residual sludge are molten with 5 kilos rosin and 2,500 of borax and, optionally, with 2,500 kg. of fluor-spar and 2,500 kilos of sodium chloride. The molten tin easily separates from its slag. The crude tin may be refined electrolytically, the anodic sludge containing all gold and silver, and also lead and bronze wastes.

I claim:

1. A method of treating bronze wastes comprising maintaining a mass of the bronze waste in a confined zone in an electrolytic bath consisting of an acidified solution of copper sulphate, maintaining a cathode in said bath, passing an electric current through said mass of bronze waste as an anode and through said bath to deposit copper on said cathode, passing a mixture of air and steam through the mass of bronze waste while in said bath, draining the bath, washing the

anode formed of bronze wastes to remove the sludge formed therein, separating copper sulphate from the sludge by washing, drying and sifting the sludge, roasting the slime at a temperature of 200-300° C., treating the roasted slime with hot dilute sulphuric acid to separate copper in the form of copper sulphate, drying and pulverizing the residue, and fusing it with a mixture of resin and molten borax for obtaining tin.

2. A method of treating bronze wastes comprising maintaining a mass of the bronze waste in a confined zone in an electrolytic bath consisting of an acidified solution of copper sulphate, maintaining a cathode in said bath, passing an electric current through said mass of bronze waste as an anode and through said bath to deposit copper on said cathode, passing air and steam through the mass of bronze waste while in said bath, draining the bath, washing the anode formed of bronze wastes to remove the sludge formed therein, separating copper sulphate from the sludge by washing, drying and sifting the sludge, roasting the slime at a temperature of 200-300° C., treating the roasted slime with hot dilute sulphuric acid to separate copper in the copper sulphate, drying and pulverizing the residue and fusing it with a mixture of resin and molten borax for obtaining tin, electrolytically refining the tin, and treating the sludge formed at the anode for the extraction of lead, silver and gold.

AUGUSTE HOLLARD.